

F. E. CANDA.  
PROCESS OF PRODUCING COMPOSITE BARS.  
APPLICATION FILED FEB. 18, 1907.

1,107,755.

Patented Aug. 18, 1914.



# UNITED STATES PATENT OFFICE.

FERDINAND E. CANDA, OF NEW YORK, N. Y., ASSIGNOR TO CHROME STEEL WORKS, OF CHROME, NEW JERSEY, A CORPORATION OF NEW JERSEY.

## PROCESS OF PRODUCING COMPOSITE BARS.

1,107,755.

Specification of Letters Patent. Patented Aug. 18, 1914.

Application filed February 18, 1907. Serial No. 357,853.

*To all whom it may concern:*

Be it known that I, FERDINAND E. CANDA, a citizen of the United States, residing at New York, in the county of New York and State of New York, have invented certain new and useful Improvements in Processes of Producing Composite Bars; and I do hereby declare the following to be a full, clear, and exact description of the same, such 10 as will enable others skilled in the art to which it appertains to make and use the same.

This invention relates to processes of producing composite bars, particularly jail bars and the like, and consists in a method of making composite jail bars and like articles comprising a body of relatively soft metal having interspersed therethrough a plurality of cores of harder metal, and specifically, in a method of making such composite jail bars or like articles having projecting ribs on their sides into which ribs certain of said hard cores extend.

In jail bars it is desirable to have a body 25 of tough and flexible character (which of course, means a relatively soft steel or like metal), containing a plurality of cores or bars of harder metal so interspersed through the mass of softer metal as to prevent sawing or boring of the bar; the soft but tough 30 metal constituting the body of the bar, preventing breaking of the bar even when the same is bent cold and permitting the bar to be shaped when either hot or cold. Such a 35 compound bar I have described and claimed in my application Sr. No. 314,032. In the case of certain types of jail bars, and of bars for other purposes, it is desirable to have on the surfaces of such bars longitudinal ribs; 40 and in such cases it is desirable that the hard cores or cast-in bars before referred to, shall extend up into such ribs so as to prevent sawing off or sawing through the ribs themselves. In the casting of the composite 45 ingots for these bars trouble has sometimes been experienced in the case of large ingots, owing to "piping," which is greatly increased over what is commonly experienced in steel casting, by the presence of the relatively cold hard steel bars. It is necessary 50 to obviate this piping as when rolling a bar with considerable piping within it the relative positions of the inserted hard metal bars may be changed materially. My present in-

vention comprises a method of reducing or 55 preventing this piping.

I have discovered that if a plurality of bars of hard metal be arranged in an ingot mold and soft steel or other soft metal cast thereabout so as to form an ingot, the ingot 60 so formed may thereafter be rolled down in the ordinary manner and the cast-in bars will nevertheless retain substantially their original relative positions and substantially 65 their original proportions with respect to the proportions of the bar itself; and in the case of the production of a ribbed bar, I have found that if in the original ingot hard steel bars be cast in edgewise in positions corresponding to the positions of the ribs in the 70 completed bar, and if the bar be rolled down in the manner hereinafter described, these edgewise cast-in hard steel cores may be drawn up into the ribs formed in the rolling 75 so that it is as impossible or difficult to saw or bore through the ribs as through the body 80 of the bar itself. Such ribs will be surrounded and supported by the softer metal, making it difficult to break them loose. I have further found that piping in large ingots such as referred to above, may be prevented by placing in the mold in a position 85 corresponding to that at which piping would otherwise occur, a bar of soft metal and causing such bar to be cast into the ingot formed.

In the accompanying drawings I illustrate the various steps in the production of the jail bars such as herein referred to.

In said drawings: Figure 1 shows a vertical longitudinal section of a mold with hard 90 metal bars therein, said mold being prepared for the pouring of the softer and tougher metal therein. Fig. 2 shows a transverse section through such a mold. Fig. 3 is a view similar to Fig. 2, but indicates the 95 use of a soft metal center rod to reduce piping. Fig. 4 shows a transverse section of one form of ingot such as may be used in the production of the jail bars, and the like. Fig. 5 shows another such form of ingot; 100 and Fig. 6 still another such form. Fig. 7 shows on a larger scale than the preceding figures, a transverse section of a ribbed jail bar constructed as herein described; and Fig. 8 shows a detail elevation of reducing 105 rolls, and illustrates the formation of the ribs thereby.

In said drawings, 1 designates the flask of

the mold, 2 the green sand body of the mold, 3, 8 dry sand cores in the mold, one of them containing the runner 4, said cores supporting the inserted hard metal bars 5.

5 The mold having been prepared, the cores inserted and the bars 5 placed within said cores, the mold is poured in the ordinary manner, the softer metal, usually low carbon steel, rising up around the inserted rods or 10 cores 5 and completely surrounding the same and welding thereto. In this way ingots of any of the sections shown in Figs. 4, 5 and 6 may be produced. In Figs. 5 and 6, 6 designates the tough metal body of the ingot, 15 and 7, 7 and 8, 8 cast-in cores or bars of harder metal, such as were originally the bars 5 inserted into the mold. For preventing piping of the ingot I place within the mold a center rod of soft metal which in the 20 final ingot produces the soft metal cast-in bar 9 indicated in Figs. 3, 5, 6 and 7.

When it is desired to form ribbed jail bars or the like, into the ribs of which hard metal cores are to be drawn, the bars which 25 are to be so drawn up into the ribs are of rectangular or other elongated cross section, and are placed edgewise or radially, so as to produce ingots such as shown in Figs. 5 and 6 for example, in which numerals 8 30 designate bars which were so placed edgewise in the mold and are still arranged edgewise in the cast ingot. In reducing these ingots to final form they are rolled in the ordinary manner except that they are 35 rolled only from the sides which these cores 8 face, and from the sides at right angles thereto. I commonly start with bars of octagonal section, though this is not essential, and work from that section to a square section 40 and then to an oval and finally to the round ribbed section, the final pass being between rolls having circular grooves 10 (Fig. 8) at the bases of which are other 45 grooves 11 corresponding to the ribs to be formed. Care is taken in this final pass that the hard metal cores 8 are presented exactly in registry with these ribbed grooves 11. The result is that in the final bar these 50 cores 8 are drawn up into the ribs 12, as indicated in Fig. 7. In this rolling, at the beginning the hard steel cores may be, and commonly are, softer than the soft steel body portion of the ingot, owing to the fact that high carbon steel melts at a lower temperature 55 than low carbon steel, and consequently at higher forging temperatures is softer than low carbon steel. Nevertheless the ingot rolls readily and without change of relative positions of the various 60 hard steel cores. As the metal cools during rolling the hard steel cores become of the same hardness as the soft steel body, and finally become of greater hardness; and it is doubtless owing to this fact, that it 65 is possible in the final pass for forming the

ribs 12, to draw the edgewise cores 8 up into these ribs, as shown in Fig. 7.

The soft metal center bars 9 doubtless prevent piping by chilling the molten metal in immediate contact with them and at the 70 same time welding thereto, thus causing solidification to start from the inside as well as from the outside, and providing a body of relatively strong metal to resist the disruptive stresses within the body of the ingot 75 due to solidification at the outside. The rolling takes out whatever internal stresses there may be in the metal due to solidification both from the outside and from the center.

80 What I claim is:—

1. The process of producing composite bars which consists in placing hard metal bars in a spaced arrangement in a mold, pouring softer metal around said bars, rolling the resulting ingot to approximate final dimensions while preserving symmetrical form, and finally rolling at a lower temperature into ribbed form, with certain of said harder metal bars opposite the positions for 90 said ribs, and thereby drawing such harder metal bars into the ribs so formed.

2. The process of producing composite ribbed bars which consists in placing hard metal bars in a spaced arrangement in a 95 mold, pouring soft metal around said bars, rolling the resulting ingot at a comparatively high temperature and thereby producing symmetrical reduction of the joined metals, and subsequently completing the reduction at a lower temperature, the bar being rolled with certain of said included hard metal bars opposite rib-forming grooves of such rolls, and by the rib-forming action of such grooved rolls drawing 100 such hard metal bars up into the ribs thus 105 formed.

3. The process of producing composite ribbed bars which consists in placing hard metal bars in a spaced arrangement in a 110 mold, certain of said bars which are to be included in the ribs when formed, being of elongated section and being placed with their edges toward the side of the mold, pouring soft metal around said bars, and 115 rolling the resulting ingot in a plurality of passes, the last pass being between grooved rib-forming rolls, with the edgewise included hard metal bars opposite the positions for the ribs, whereby such hard metal 120 bars are drawn up into the ribs so formed.

4. The process of producing composite ribbed bars which consists in placing hard metal bars in a spaced arrangement in a 125 mold, certain of said bars which are to be included in the ribs when formed, being of elongated section and being placed with their edges toward the side of the mold, pouring soft metal around said bars, and 130 rolling the resulting ingot in a plurality of

passes on the sides nearest such edgewise turned bars, and on the sides at right angles thereto, the final pass being between grooved rib-forming rolls, with the edgewise included hard metal bars opposite the positions for the ribs, whereby such hard metal bars are drawn up into the ribs so formed.

5. The herein described process of producing composite jail bars and the like, which consists in placing in a suitable mold in spaced arrangement a series of cores of hard metal, said cores relatively arranged in the outline of a closed figure inclosing a central space, pouring molten softer metal

10 into said mold and about said bars and within the space inclosed thereby, and finally working down the ingot so formed.

15

6. The herein described process of producing composite jail bars and the like, which consists in placing in a suitable mold 20 a series of cores of hard metal in a spaced arrangement in the form of a closed figure inclosing a central space, and further placing in the mold a soft metal bar in a position approximating the center of the ingot to be 25 formed, pouring softer metal into said mold and about said bars, and finally working down the ingot so formed.

In testimony whereof I affix my signature, in the presence of two witnesses.

FERDINAND E. CANADA.

Witnesses:

ALPHONSE KLOH,  
H. M. MARBLE.